

## UNITED STATES PATENT OFFICE.

STANLEY TUCKER, OF LONDON, AND EDWIN EDSER, OF BROCKLEY, LONDON, ENGLAND,  
ASSIGNORS TO MINERALS SEPARATION NORTH AMERICAN CORPORATION, OF NEW  
YORK, N. Y.

## CONCENTRATION OF ORES.

No Drawing.

Application filed November 20, 1919. Serial No. 339,384.

*To all whom it may concern:*

Be it known that we, STANLEY TUCKER, a subject of the King of England, residing at London, England, and EDWIN EDSER, a subject of the King of England, residing at Brockley, London, England, have invented certain new and useful Improvements in the Concentration of Ores, of which the following is a specification.

10 This invention relates to improvements in the concentration of ores, and it refers more particularly to flotation separation, such as by the froth-flotation process described, for example, in the prior United States Patents 15 Nos. 835,120 to Sulman, Picard and Ballot, dated November 6, 1906, 962,678 to Sulman, Greenway and Higgins, dated June 28, 1910, 1,064,723 to Greenway and Lavers, dated June 17, 1913, and application of Sulman 20 and Edser, Serial No. 162,320, filed April 16, 1917.

The froth flotation process of concentrating ores as described in these prior specifications consists in agitating and/or aerating 25 the crushed ore in water to which is added a minute proportion of a mineral-frothing agent for the formation of a froth carrying the metalliferous particles which is allowed to float on the surface of the liquid separate 30 from the gangue particles, whence it is removed.

It has previously been proposed to treat 35 oxidized metalliferous particles with soluble sulphides or sulphuretted hydrogen for the purpose of coating with or converting into sulphide the oxide particles so as to render them capable of separation by the froth-flotation process; a small quantity of a soluble sulphide has also been added to the ore 40 pulp when treating a mixed sulphide ore for the purpose of obtaining a froth carrying certain of the particles in preference to other particles.

In the prior Patent No. 1,236,857 to Martin dated August 14, 1917, it has been proposed to use a mineral-frothing agent consisting of or containing an oil which has been heated in the presence of sulphur, and in said prior application Serial No. 162,320 50 the employment as the mineral-frothing agent of a soluble soap, such as sodium

oleate, sodium stearate, sodium palmitate or sodium resinate, has been described.

It has now been found that there may be used as a mineral-frothing agent the fairly 55 stable product obtained by adding to a solution of a soap, such as sodium oleate, a solution of an alkaline sulphide or sulphhydrate; or by treating the solution of an alkaline sulphide with a fatty acid; or by mixing or 60 combining materials or ingredients necessary to produce soluble soaps and alkaline sulphides, as for example by treating an alkaline hydrate or carbonate with sulphur and adding a fatty acid; or by treating a solution of an alkaline sulphide containing sulphur in excess of the normal sulphide with a fatty acid; or by adding a soluble soap to an aqueous solution of sulphuretted 65 hydrogen.

When treating an alkaline sulphide with a fatty acid or mixing or combining materials or ingredients necessary to produce soluble soaps and alkaline sulphides, the 70 quantities thereof should preferably be such as to produce a solution which still contains some alkaline hydrosulphide, sulphide or polysulphide, or sulphuretted hydrogen. It is to be understood that if some sulphur or sulphuretted hydrogen is liberated during 75 the preparation of the above, this will not necessarily prevent the formation of a froth-forming reagent of peculiar efficiency.

Soluble soaps which are suitable for use 80 in the present invention are the alkali compounds of the fatty or resin acids. That is they contain an acid soap-forming radical, and an alkali radical while the sulphur or sulphur compound furnishes a sulphide radical.

The following are examples of the preparation of products suitable for mineral-frothing agents according to the present invention.

*Example I.*—46.5 grammes of oleic acid 85 were added to a boiling solution of 20 grammes of crystallized sodium sulphide ( $Na_2S \cdot 9H_2O$ ), in about 600 ccs. of water, and the clear or homogeneous solution obtained was diluted to 1 litre. Very little 90 sulphuretted hydrogen was given off during the reaction.

*Example II.*—22 grammes of oleic acid were added to a hot solution prepared by boiling two grammes of sulphur in a solution of 20 grammes of sodium sulphide crystals in about 600 ccs. of water.

*Example III.*—22 grammes of oleic acid were added to a hot solution made by boiling 2 grammes of sulphur with 23 grammes of crystalline sesqui-carbonate of soda in about 600 ccs. of water. In this case some of the sulphur did not go into solution.

The following is an example of the use of the products prepared as described above in the froth-flotation process of concentrating ores, a differential separation being obtained:—

500 grammes of an ore from a Peruvian mine containing 17.6% Pb as galena and 20 34% Zn as blende, crushed to 80 mesh, was made into 5:1 pulp with soft water containing 0.25% of liquid sodium silicate (140° Twaddell). 16 ccs. of the product prepared as described in Example I above 25 was added and the mixture was aerated by the sub-aeration method. A froth was formed, the solid contents of which weighed 112 grammes and assayed 60% Pb and 12.2% Zn, giving a recovery of 76.5% Pb 30 and 8% Zn. The tailings contained 5.35% Pb and 40.3% Zn.

In an exactly parallel test with the same ore using 16 ccs. of a 5% solution of sodium oleate, a froth was formed the solid contents of which weighed 121 grammes and assayed 48% Pb and 19% Zn, giving a recovery of 66% Pb and 13.8% Zn. The tailings assayed 7.9% Pb and 38% Zn.

The product obtained as described above 40 may be employed as a mineral-frothing agent not only in the differential separation of certain metalliferous particles from other metalliferous particles in a mixture containing them, but also in the concentration of sulphide ores and oxidized ores.

As an example of the concentration of an oxidized ore:

400 grammes of wolframite ore containing tungsten equal to 4.1% of  $WO_3$  was 50 agitated with 1600 ccs. of soft water to which was added sodium silicate solution equivalent to 1 lb. of sodium silicate per ton of ore as a modifying agent, and 16 ccs. of a solution prepared as in Example 55 I. The mixture was then agitated and aerated by sub-aeration for the formation of a froth. The solid contents of the froth weighed 86 grammes and assayed tungsten equivalent to 16.8%  $WO_3$ . The tailings 60 weighed 314 grammes and assayed tungsten equivalent to 0.55%  $WO_3$ . Thus a recovery equivalent to 88% of the wolframite was obtained.

The product described above is efficient 65 for the separation of cassiterite from tin-

bearing ores, in which case the addition of a small quantity of acid, for example one-half pound per ton of ore of sulphuric acid, may sometimes be desirable.

The same procedure is also applicable to 70 oxidized ores of copper and lead and other metals, but it is to be understood that the presence of acid may not always be necessary.

In some cases it is preferable that the 75 materials described above should be freshly prepared.

What we claim as our invention and desire to secure by Letters Patent is:—

1. The process of concentrating ores which 80 consists in mixing with an ore pulp a mineral-frothing agent obtained by causing a reaction to be effected between substances containing a soap-forming acid radical, an alkaline radical, and a sulphide radical to 85 produce the agent and also bringing gaseous bubbles into contact with the solid particles in the ore pulp so as to produce mineral-bearing froth, and separating the froth.

2. The process of concentrating ores which 90 consists in mixing with an ore pulp a mineral-frothing agent obtained by causing a reaction to be effected between ingredients adapted to produce soluble soaps and alkaline sulphides when mixed, and also bringing 95 gaseous bubbles into contact with the solid particles in the ore pulp so as to produce mineral-bearing froth, and separating the froth.

3. In the froth-flotation process of 100 concentrating ores the employment as a mineral-frothing agent of the product obtained by treating a fatty acid with a solution of an alkali which has previously been treated with sulphur.

4. The process of concentrating ores which 105 consists in mixing with an ore pulp a mineral-frothing agent obtained by causing a reaction to be effected between ingredients adapted to produce a substantially homogeneous composition adapted to go into solution and containing in stable combination soap material and sulphur, and also bringing 110 gaseous bubbles into contact with the solid particles in the ore pulp so as to produce mineral-bearing froth, and separating the froth.

5. The process of concentrating ores which 115 consists in mixing with an ore pulp a mineral-frothing agent obtained by causing a reaction to be effected between ingredients adapted to react to produce soluble soap and alkaline sulphides, so that the solution still contains additionally a soluble compound containing a sulphide radical, and also bringing 120 gaseous bubbles into contact with the solid particles in the ore pulp so as to produce mineral-bearing froth, and separating the froth.

6. The process of concentrating ores which 125

consists in mixing with an ore pulp a mineral-frothing agent obtained by causing a reaction to be effected between ingredients adapted to react to produce a clear solution

5 of substances containing a soap-forming acid radical, an alkaline radical, and a sulphide radical, and also bringing gaseous bubbles into contact with the solid particles in the ore pulp so as to produce mineral-bearing

10 froth, and separating the froth.

7. The process of concentrating ores which consists in mixing with an ore pulp a mineral-frothing agent obtained by causing a reaction to be effected between ingredients 15 adapted to react when boiled together in aqueous mixture to produce a clear solution of substances containing a soap-forming acid radical, an alkaline radical, and a sulphide radical, and also bringing gaseous bubbles 20 into contact with the solid particles in the ore pulp so as to produce mineral-bearing froth, and separating the froth.

8. The process of concentrating ores which consists in mixing with an ore pulp a mineral-frothing agent obtained by causing a reaction to be effected between ingredients 25 adapted to react when boiled together in aqueous mixture to produce soluble soap and alkaline sulphides, so that the solution still 30 contains additionally a soluble compound containing a sulphide radical, and also bring-

ing gaseous bubbles into contact with the solid particles in the ore pulp so as to produce mineral-bearing froth, and separating the froth.

35

9. The process of concentrating ores which consists in mixing with an ore pulp a mineral-frothing agent obtained by causing a reaction to be effected between ingredients when boiled together in aqueous mixture 40 adapted to produce a substantially homogeneous composition adapted to go into solution and containing in stable combination soap material and sulphur, and also bringing gaseous bubbles into contact with the 45 solid particles in the ore pulp so as to produce mineral-bearing froth, and separating the froth.

10. The process of concentrating ores which consists in mixing with an ore pulp a 50 mineral-frothing agent obtained by causing a reaction to be effected by boiling together a soap-forming acid radical and material containing a sulphide radical to produce the agent, and also bringing gaseous bubbles into 55 contact with the solid particles in the ore pulp so as to produce mineral-bearing froth, and separating the froth.

In testimony whereof we have signed our names to this specification.

STANLEY TUCKER.  
EDWIN EDSER.